



US007430797B2

(12) **United States Patent**  
**Peinsipp et al.**

(10) **Patent No.:** **US 7,430,797 B2**  
(b4) **Date of Patent:** **Oct. 7, 2008**

(54) **METHOD FOR MAKING AN ELECTRICAL COMPONENT**

(75) Inventors: **Roland Peinsipp**, Graz (AT); **Franz Schrank**, Raaba (AT)

(73) Assignee: **EPCOS AG**, Munich (DE)

(\*) Notice: Subject to any disclaimer, the term of this patent is extended or adjusted under 35 U.S.C. 154(b) by 23 days.

(21) Appl. No.: **11/586,969**

(22) Filed: **Oct. 25, 2006**

(65) **Prior Publication Data**

US 2007/0040646 A1 Feb. 22, 2007

**Related U.S. Application Data**

(62) Division of application No. 10/363,275, filed on May 30, 2003, now Pat. No. 7,145,430.

(30) **Foreign Application Priority Data**

Aug. 30, 2000 (DE) 100 42 636

(51) **Int. Cl.**

**H01C 17/02** (2006.01)

(52) **U.S. Cl.** 29/613; 29/612; 29/619; 29/842; 338/22 R

(58) **Field of Classification Search** 29/592.1, 29/595, 610.1, 612, 613, 619, 621, 842; 338/22 R, 338/22 SD, 21, 25, 156, 257

See application file for complete search history.

(56) **References Cited**

U.S. PATENT DOCUMENTS

2,741,687 A 4/1956 Toppari  
2,883,502 A 4/1959 Rudner

|                |         |                          |
|----------------|---------|--------------------------|
| 2,885,523 A    | 5/1959  | Wright et al.            |
| 3,562,007 A *  | 2/1971  | Bockstie et al. 428/215  |
| 3,599,139 A    | 8/1971  | Low                      |
| 3,655,610 A    | 4/1972  | Vasta                    |
| 3,666,551 A    | 5/1972  | Bockstie, Jr.            |
| 3,793,716 A    | 2/1974  | Smith-Johannsen          |
| 3,824,328 A *  | 7/1974  | Ting et al. 174/524      |
| 4,001,655 A    | 1/1977  | Voyles et al.            |
| 4,959,426 A    | 9/1990  | Re et al.                |
| 5,321,386 A *  | 6/1994  | Ishiguro 338/269         |
| 5,661,618 A *  | 8/1997  | Brown et al. 360/97.02   |
| 6,025,556 A *  | 2/2000  | Yoshimura et al. 174/524 |
| 6,800,176 B1 * | 10/2004 | Birchenall 162/164.1     |

FOREIGN PATENT DOCUMENTS

|    |            |         |
|----|------------|---------|
| DE | 25 00 789  | 7/1975  |
| DE | 23 51 956  | 12/1982 |
| DE | 37 89 365  | 9/1994  |
| DE | 198 14 388 | 10/1998 |
| DE | 198 51 869 | 7/2000  |
| DE | 197 21 101 | 3/2004  |
| EP | 0322339    | 6/1989  |
| JP | 1-235203   | 9/1989  |

\* cited by examiner

Primary Examiner—Donghai D. Nguyen

(74) Attorney, Agent, or Firm—Schiff Hardin LLP

(57) **ABSTRACT**

An method for manufacturing an electrical component comprises providing a base body of a ceramic material with at least two contact regions with terminal elements secured thereto. The base body is immersed into a solution that contains a fluid that wets the base body and a hydrophobic and lipophobic intermediate layer material dissolved in the fluid. The base body is removed from the solution so that a part of the solution remains adhering thereto as a film that completely envelopes the base body. An intermediate layer is produced by evaporating the fluid contained in the film, and a protective layer is applied onto the intermediate layer.

**4 Claims, 1 Drawing Sheet**





## 1

METHOD FOR MAKING AN ELECTRICAL  
COMPONENTCROSS-REFERENCE TO RELATED  
APPLICATIONS

This application is a divisional of parent application Ser. No. 10/363,275, filed May 30, 2003, Issued as U.S. Pat. No. 7,145,430. The parent application is herein incorporated by reference.

## BACKGROUND

The invention is directed to an electrical component having a base body that comprises a ceramic material and having at least two contact regions arranged in the base body to which terminal elements are secured. The component is enveloped with a protective layer containing organic constituents. The invention is also directed to a method for the manufacture of the electrical component.

German patent document DE 198 51 869 A1 discloses electrical components of the species initially cited that represent a hot-carrier thermistor temperature sensor composed of a disk-shaped ceramic material. In addition to leads attached to the material, the temperature sensor comprises an epoxy resin envelope that contains an auxiliary constituent with hydrophobic properties.

The known electrical component has the disadvantage that it is sensitive to moisture. Even though it has a hydrophobic envelope of epoxy resin that, for example, can be produced by immersion, outages can occur under the influence of moisture and/or water as a consequence of migration effects. Due to the adjacent voltage employed in the operation of the component, namely, there is a difference in potential between the two electrical poles of the ceramic element to which the leads are secured. When, under the use conditions in a humid environment, a closed water film forms between the electrodes, then a material transport starts (mediated by silver, tin and lead of the solder employed when soldering the leads on) from the anode to the cathode. Metallic films are formed that are capable of functioning similar to interconnects on the surface of the ceramic. The resistance of the sensor therefore decreases so greatly that a total outage of the hot-carrier thermistor temperature sensor can even occur under certain circumstance due to a short. Such hot-carrier thermistor temperature sensors can therefore only be provided for areas of employment wherein a moistening or, respectively, an influence of water at the temperature sensor does not occur.

In order to avoid the described problem, it is known from the Prior Art to provide the hot-carrier thermistor temperature sensor with a glass envelope. Given this design, however, no insulated leads can be utilized due to the high process temperatures. Moreover, there is a risk here that damage due to electro-chemical corrosion of the wires or migration via the glass member can occur given corresponding use conditions.

## SUMMARY OF THE INVENTION

It is therefore an object of the present invention to specify a component of the species initially cited that exhibits a long service life even under the influence of moisture.

This object is inventively achieved by an electrical component having a base body that comprises a ceramic material and has at least two contact regions arranged in the base body to which terminal elements are secured, and this component is enveloped with a protective layer containing organic constituents, and has an intermediate layer that is arranged between

## 2

the base body and the protective layer and is composed of an intermediate layer material that is both hydrophobic as well as lipophobic.

The component has the advantage that, due to the intermediate layer of hydrophobic material, the penetration of moisture from the outside onto the surface of the base body can be effectively reduced at those locations at which the base body is covered by the intermediate layer.

In addition, the inventive component has the advantage that, due to the lipophobic material property of the intermediate layer, this is compatible with the protective layer surrounding the base body. In particular, no chemical reaction occurs between the protective layer and the intermediate layer. As a result thereof, a migration of constituents of the protective layer through the intermediate layer onto the surface of the base body can also be effectively prevented, including the damage that becomes possible as a result thereof.

It is especially advantageous when the intermediate layer tightly surrounds the base body of the component, so that access of moisture is inhibited at the entire surface of the base body.

In addition, a component is especially advantageous wherein the intermediate layer material is soluble in a fluid with which the base body can be moistened.

Such a component has the advantage that the intermediate layer can be produced in a simple way by immersing the base body into a solution that contains the fluid and the intermediate layer material dissolved therein.

As a result thereof, the base body can be moistened by the fluid, and the advantage derives that the base body can be unproblematically covered with the intermediate layer so that the intermediate layer tightly surrounds the base body.

In addition, a component is especially advantageous wherein the thickness of the intermediate layer amounts to at least 1.5  $\mu\text{m}$  at its thinnest location. This minimum thickness guarantees that the access of moisture to the base body is inhibited at all locations at which the intermediate layer is arranged on the base body.

For example, a fluoropolymer is a material suitable for the intermediate layer that exhibits the required properties. This is thereby a matter of a perfluorinated carbon framework structure. The carbon framework structure can thereby be constructed of chains, of connected ring systems or of a mixed form of the two. In particular, an intermediate layer material is especially advantageous that is formed of condensed perfluorinated ring systems. Further, polyethers are also employable that comprise no C—C chains but C—O—C chains. The molecular weight of the polymer advantageously lies above 1000 g/mol. A fluoropolymer is also advantageous that is soluble in specific solvents, preferably in perfluorinated alkanes.

The fluorine-containing polymer can also have the advantage that it exhibits a soft, wax-like consistency that can have a favorable influence on the thermal fatigue resistance of the layer and of the entire component as well.

The protective layer of the component can thereby be advantageously composed of a material that is electrically insulating and is simultaneously suited for protecting the intermediate layer against abrasion. A protective layer of this material has the advantage that it protects the component from electrical shorts from the outside. In addition, the protective layer has the advantage that it can effectively protect the intermediate layer against mechanical damage due, for example, to abrasion, so that the intermediate layer can be composed of a fluoropolymer that can have a low mechanical resistance and exhibit a soft, wax-like consistency.

A protective layer that exhibits the demanded properties with respect to the electrical insulation and the protection of the intermediate layer is advantageously composed of epoxy resin, silicone or urethane.

The invention also specifies a method for the manufacture of an electrical component that is based on a base body that comprises a ceramic material. The base body thereby comprises at least two contact regions to which terminal elements are secured.

The method comprises the following steps:

In a first step, the base body is immersed into a solution that contains a fluid that wets the base body and a hydrophobic and lipophobic intermediate layer material dissolved in this fluid. Advantageously, the base body is thereby immersed into the solution so that the base body is situated entirely within the solution.

In a further step, the base body is removed from the solution so that a part of the solution remains adhering thereto as a film that completely envelopes the base body.

In a further step, the fluid contained in the film is removed by evaporation, and the intermediate layer occurs as a result of the evaporation.

In a following step, the protective layer is applied onto the intermediate layer. The protective layer can also be advantageously applied by immersing the base body into a corresponding solution or, respectively, fluid.

The inventive method for manufacturing the electrical component has the advantage that it is especially simple to realize since the base body of the component merely has to be immersed into a solution for the application of the intermediate layer. In addition, the method has the advantage that the manufacture of the intermediate layer from the solution occurs by evaporation of fluid in a fluid film. Such an evaporation requires no further technical measures other than simple storing of the component at, for example, room temperature and can thus be cost-beneficially realized.

The method can be especially advantageously implemented in that the viscosity of the solution into which the base body is immersed is set by means of a suitable selection of the content of the intermediate layer material in the solution that the film adhering to the base body leads to an intermediate layer that is at least 1.5 µm thick at the thinnest location. This measure assures that the intermediate layer comprises the required minimum thickness at every location.

A perfluoro alkane in which a fluoropolymer, which is suitable as an intermediate layer material, is soluble can be advantageously employed as the fluid that contains the intermediate layer material in a dissolved form.

The invention is explained in greater detail below on the basis of an exemplary embodiment and the appertaining FIGURE.

#### BRIEF DESCRIPTION OF THE DRAWING

The FIGURE shows a schematic cross-section of an inventive electrical component by way of example.

#### DESCRIPTION OF THE PREFERRED EMBODIMENTS

The FIGURE shows an electrical component having a base body 1 that can be composed of a polycrystalline ceramic of the spinel type, particularly the Mn—Ni spinel type, and that can, over and above this, contain additional dopings or, respectively, secondary constituents. Additionally, ceramics are also conceivable that are composed of other principal constituents. The aforementioned ceramic of the Mn—Ni

spinel type is usually employed as the base body 1 for hot-carrier thermistor temperature sensors. It is especially important precisely in such hot-carrier thermistor temperature sensors that the base body exhibit a stable electrical resistance 5 that is not changed due to the influence of moisture.

The FIGURE also shows a first contact region 2 and a second contact region 3 that are applied to the upper side or, respectively, underside of the base body 1. These contact regions can, for example, be manufactured by means of a 10 silver stoving paste. A first terminal element 4 that, for example, can be a wire provided with an electrical insulation is secured to the first contact region 2. The fastening of such a wire to the first contact region 2 preferably occurs by soldering. In the same way as at the first contact region 2, a 15 second terminal element 5 in the form of an insulated wire that is soldered on and is secured to the second contact region 3.

The base body 1 is enveloped by an intermediate layer 7 that is applied by immersing the base body 1 into a solution of 20 a fluoropolymer. This fluoropolymer is constructed of multi-cyclic monomer units and its molecular weight amounts to approximately 2000 g/mol. The concentration of the solution of this polymer lies between 1% and 30%. The viscosity of the solution can be set by the concentration of the solution, so that 25 the thickness of the intermediate layer 7 is also defined as a result thereof. For example, easily obtainable perfluoroalkanes, particularly perfluorohexane or perfluorooctane, are suitable as a solvent.

After the solvent is dried off, the envelope is enveloped 30 with a two-component epoxy in an immersion process. The protective layer 6 is formed as a result of this step.

It should be noted with respect to the intermediate layer 7 that, due to the application of the layer in an immersion process, a largely uniform layer thickness as shown in the 35 FIGURE cannot be achieved. On the contrary, the layer at the edges of the base body 1 will be significantly thinner than, for example, between the contact regions 2, 3. In the exemplary embodiment described here, an intermediate layer 7 was produced that can comprise a layer thickness of less than 2 µm at 40 the edges of the base body 1 and thicknesses up to 5 µm at other locations.

The protective layer 6 is applied by means of the described immersion process and it comprises a layer thickness between 100 µm and 1000 µm. That stated for the intermediate layer 7 applies to the protective layer 6 with respect to its thickness. All standard envelope materials, for example on the basis of epoxy resin, that are electrically insulating and exhibit a minimum resistance to the formation of cracks come into consideration as the protective layer 6. In addition to 45 epoxy resin, polyurethane resin or silicone lacquer also come into consideration. In addition to being applied in the immersion process, the protective layer 6 can also be applied with some other method, for example with a powder coating method.

When manufacturing the intermediate layer 7 or, respectively, the protective layer 6, the base body 1 is preferably 50 immersed into the corresponding fluid so that end sections 8, 9 of the terminal elements 4, 5 remain uncoated and can thus be employed as electrical contacts for connecting the component in a circuit.

A temperature sensor manufactured according to the 55 described exemplary embodiment was tested for water resistance under various test conditions. For that purpose, for example, a storing in water at a temperature of 80° and an adjacent d.c. voltage of 3 V was implemented over 2000 hours. The temperature sensor passed this test without any 60 change in the electrical resistance.

## 5

Other tests that were implemented, which contain a succession of various types of loads such as, for example: thermal cycling, followed by vibration, subsequent storing in water at a temperature of 80° and an adjacent d.c. voltage of 3 V, followed by electrical loading with a heating capacity of 60 mW, subsequent cyclical moistening or, respectively, ice-coating upon application of an electrical voltage, as well as following aging at a temperature of 155° C. and subsequent storing of the temperature sensor in water at 80° C. upon application of a voltage of 3 V. The temperature sensor also passed this sequence of stresses without damage. The tests were passed without the temperature sensor having changed in electrical resistance.

The same tests were implemented with a similar temperature sensor but without the intermediate layer 7. 100% of such temperature sensors had already failed after fewer than 100 hours given storing in water at 80° C. upon application of an electrical voltage of 3 V.

The invention is not limited to the illustrated exemplary embodiment but is defined in its broadcast form by the claims.

The invention claimed is:

1. A method for manufacturing an electrical component, comprising:

## 6

providing a base body of a ceramic material with at least two contact regions with terminal elements secured to the two contact regions;

immersing the base body into a solution that contains a fluid that wets the base body and an intermediate layer material dissolved in the fluid that comprises a fluoropolymer or a polyether;

removing the base body from the solution so that a part of the solution remains adhering thereto as a film that completely envelopes the base body, the two contact regions and part of the terminal elements

producing an intermediate layer by evaporating the fluid contained in the film; and

applying a protective layer onto the intermediate layer.

15 2. The method according to claim 1, wherein the fluid is a perfluoroalkane and the intermediate layer material is a fluoropolymer.

3. The method according to claim 1, wherein the solution has processing properties that are selected so that the film 20 adhering to the base body leads to said intermediate layer being at least 1.5  $\mu$ m thick at its thinnest location.

4. The method according to claim 3, wherein the fluid of the solution is a perfluoroalkane and the intermediate layer material is a fluoropolymer.

\* \* \* \* \*